

# UNITED STATES PATENT OFFICE.

NICOLAS C. ARMAND AND JACQUES E. BERTON, OF PARIS, FRANCE.

## DYEING FABRICS WITH ANILINE COLORS.

SPECIFICATION forming part of Letters Patent No. 242,855, dated June 14, 1881.

Application filed January 31, 1881. (No specimens.) Patented in France December 29, 1880.

To all whom it may concern:

Be it known that we, NICOLAS CHARLES ARMAND and JACQUES EUGENE BERTON, both of Paris, in the Republic of France, have invented certain new and useful Improvements 5 in Dyeing Fabrics with Aniline Colors, of which improvements the following specification is a full description.

The invention has for its object to dye by 10 what may be called a "dry process"—that is to say, a process in which water is not employed, but only benzines and essences of mineral or vegetable origin; and it consists, essentially, in the means, as hereinafter described, for rendering the coloring-matters of aniline and its derivatives soluble in the said benzines and essences.

The improved process can be carried on at ordinary temperatures.

20 Heretofore, even with the aid of alcohol, success in dissolving the coloring-matters derived from coal-tar in benzines and mineral essences has not been attained in an industrial way.

25 In order to overcome the difficulty due to this insolubility of the compounds, and generally considered insurmountable, there is in the present invention, combined with the color as an intermediary, a special solvent which 30 possesses the desired property of rendering the same soluble in the liquids named. This solvent is composed of two distinct classes of elements, to wit: first, vegetable oils or fats; and, second, chemical compounds or reagents, 35 acetic or hydrochloric acid, sulphuric ether, volatile alkali, (ammonia,) and potash. These elements are mixed in the following proportions: oil (olive-oil, for example) or fat, (lard, for example,) forty-five parts; acetic or hydro-

40 chloric acid, twenty-five parts; sulphuric ether, seven parts; volatile alkali, seven parts; potash, sixteen parts. These proportions can be varied within certain limits, according to the colors or shades, more or less decided, which it 45 is desired to obtain. The solvent having been prepared in a suitable vessel over a slow fire, the aniline color is added in the proportion required for the desired depth of shade. A sort of paste is thus formed, which has the property of being

50 soluble in all proportions in the benzines or essences. The tinctorial product thus obtained, after becoming cold, is put into the benzine or essence, the quantity of which is regulated by the quantity of fabrics or goods to be dyed.

55 Into the coloring-bath thus prepared the fabrics are plunged and worked or rubbed, so as to cause the penetration of the liquid until the desired shade is obtained. The fabrics are then wrung out and dried in any ordinary or suitable way—that, for example, used in the process for 60 cleaning with benzine, called "dry cleaning process." In this way, therefore, threads or fabrics of silk, cotton, or mixtures of silk and cotton, can be dyed without wetting, or, in other words, without any alteration in the fiber. 65

In dyeing wool by this invention the composition of the solvent is preferably modified by substituting for five of the forty-five parts of oil or fat five parts of oleic acid, and for five of the twenty-five parts of acetic or hydrochloric acid five parts of phenic acid. 70

75 The preparation of aniline colors with a solvent which renders them soluble in benzines and essences enables the same to be advantageously employed for printing upon fabrics, and notably on those of cotton. Thus, in accordance with this invention, it is possible to dye or print with aniline colors of all shades upon yarns or threads of silk, cotton, or mixtures of silk and cotton, whether in the form 80 of skeins, fabrics, stuffs of various kinds, or made-up clothing, however made, and without injury to the same. Colors of all shades can also be obtained upon furniture, fancy articles, skins, gloves, and shoes. 85

We claim—

1. The herein-described method of rendering aniline colors soluble in benzines and essences, by combining said colors with a solvent or intermediary agent, such as the composition of oil or fat, acid, ether, and alkalies set forth. 90

2. A composition paste of aniline color and a solvent, such as the compound of oil or fat, acid, ether, and alkali set forth, adapted to render the said color soluble in benzine and essences, substantially as described. 95

3. The compound of aniline color, oil or fat, acetic or hydrochloric acid, sulphuric ether, volatile alkali, and potash, as set forth. 100

In witness whereof we have hereunto signed our names in the presence of two subscribing witnesses.

NICOLAS CHARLES ARMAND.  
JACQUES EUGENE BERTON.

Witnesses:

ROBT. M. HOOPER,  
CHARLES MARDELET.